

Patented Sept. 8, 1936

2,053,421

# UNITED STATES PATENT OFFICE

2,053,421

## CRACKED DISTILLATES OF PETROLEUM

Robert E. Burk and Herman P. Lankelma, Cleveland, Ohio, assignors, by mesne assignments, to E. I. du Pont de Nemours & Company, Wilmington, Del., a corporation of Delaware

No Drawing. Application August 7, 1930,  
Serial No. 473,775

3 Claims.

(Cl. 44—9)

This invention relates to the improvement of cracked petroleum distillates, and more particularly cracked naphthas for motor fuels. As is well known, cracked distillates have an inherent tendency to develop more or less gum formation and also go off color. In motor fuels, this is objectionable, and where gumming of the valves occurs may be serious. It is among the objects of this invention to inhibit such detrimental tendencies in cracked distillates, and in a manner facilitating manufacturing process in accordance with desirable practice.

To the accomplishment of the foregoing and related ends, the invention, then, consists of the features hereinafter fully described, and particularly pointed out in the claims, the following description setting forth in detail certain embodiments of the invention, these being illustrative however of but a few of the various ways in which the principle of the invention may be employed.

In accordance with the invention, a cracked petroleum distillate such as is prone to develop gum formation is subjected to the action of a dihydroxy derivative of a condensed nucleus hydrocarbon or a derivative in which the two hydroxyl groups are preserved, such compounds as 1,5 dihydroxy naphthalene, and 1,2 dihydroxy anthraquinone being particularly desirable.

Such agents, individually or in mixture of two or more, may be incorporated in the cracked distillate to be treated. The amount required is small, for instance 0.0004 to 0.5 per cent. In general, it is not necessary to exceed one-half of one per cent., or at the maximum one per cent., since excessive amounts are merely wasted. A desirable manner of incorporating the material into the petroleum distillate may involve first dissolving the agent in a suitable solvent, for instance ether, benzol, etc., and this solution may then be mixed with the distillate. The petroleum distillate may have been previously subjected to the customary lye wash if desired, and a slight alka-

line or at least a neutral reaction of the distillate is advantageous. The mixing may be effected in any convenient manner, as for instance adding the agent to the distillate in a container and agitating to thorough dissemination, or proportionally feeding into a stream of the petroleum distillate, thereby mixing in transit.

Example.—20 lbs. of 1,5 dihydroxy naphthalene is dissolved in benzol to make up substantially 10 gallons volume, and this is mixed with 2500 barrels of cracked gasoline.

Similarly, any of the various agents contemplated can be incorporated, and cracked distillates be so treated, for the production of motor fuels etc., which may be stored and used, with control of the gumming and discoloration tendencies otherwise objectionably occurring.

Other modes of applying the principle of the invention may be employed instead of the details disclosed, change being made as regards such details, provided the features stated in any of the following claims, or the equivalent of such, be employed.

We therefore particularly point out and distinctly claim as our invention:—

1. A cracked gasoline normally tending to develop gummy substances upon storage and containing a dihydroxy anthraquinone compound in quantity sufficient to retard such gum formation.

2. A cracked gasoline normally tending to develop gummy substances on storage and having incorporated therein in an amount sufficient to inhibit such gum formation dihydroxy anthraquinone.

3. A cracked gasoline normally tending to develop gummy substances on storage and having incorporated therein in an amount sufficient to inhibit such gum formation 1,2 dihydroxy anthraquinone.

ROBERT E. BURK.  
HERMAN P. LANKELMA.